

3,272,743

## LUBRICANTS CONTAINING METAL-FREE DISPERSANTS AND METALLIC DISPERSANTS

George R. Norman, Lyndhurst, and William M. Le Suer, Cleveland, Ohio, assignors to The Lubrizol Corporation, Wickliffe, Ohio, a corporation of Ohio  
No Drawing. Filed Aug. 5, 1964, Ser. No. 387,757  
12 Claims. (Cl. 252—32.5)

This application is a continuation-in-part of earlier application Ser. No. 77,842, filed December 23, 1960, now forfeited, which was a continuation-in-part of earlier filed application Ser. No. 808,903, filed April 24, 1959, now abandoned, which was in turn a continuation-in-part of earlier filed application Ser. No. 802,667, filed March 30, 1959, now U.S. 3,172,892.

This invention relates to a combination of chemical compositions which are especially useful in lubricants. It relates in particular to lubricating compositions containing this combination of compositions.

There are two principal environments which are served by automotive crankcase lubricants. Each of these environments poses a specific problem which must be solved if a lubricant is to be regarded as satisfactory. These problems are the result of the inevitable presence in the lubricant of varying proportions of foreign particles such as dirt, soot, water and decomposition products resulting from breakdown of the oil. Even if there were none of this latter contaminant present, the very nature of the design of the modern internal combustion engine is such that a significant amount of foreign matter will accumulate in the crankcase. Perhaps the most important of these contaminants is water because it seems to be responsible for the deposition of a mayonnaise-like sludge. It appears that if there were no water present, the solid components of the mayonnaise-like sludge would circulate with the oil and be removed by the oil filter. It will be readily appreciated that the deposition of the sludge presents a serious problem with respect to the efficient operation of the engine and that it is desirable to prevent such deposition of sludge-like material.

The presence of water and the precursors of sludge in a lubricating oil is dependent largely upon the operating temperature of the oil. If the oil is operated at a high temperature the water of course will be eliminated by evaporation about as fast as it accumulates. In the absence of water, as stated above, the other foreign particles will be removed by the filter. At low oil temperatures, on the other hand, water will accumulate and so consequently will sludge. It is apparent that this particular environment provides a serious problem for crankcase lubricants.

In ordinary stop-and-go driving, as is the case with taxicabs, delivery trucks, police cruisers, etc., the crankcase lubricant will be alternately hot and cold, an ideal environment for the accumulation of water. In such cases the formation of sludge is a serious problem. This problem has been with the automotive industry for many years and its solution has been sought by the use of many different types of additives, but without notable success. Although many of such additives are very effective in combating the detergency problems associated with motor oils at high temperatures, they have not been particularly effective in solving the problems associated with low temperature operation, or to put it better, those problems which are associated with crankcase lubricants in engines which are operated at alternating high and low temperatures.

The other principal problem which must be solved by a satisfactory lubricant is that posed by the operation of an engine at continuous high temperatures. This is the situ-

ation caused by high speed operation such as all-day driving at speeds of 50-70 m.p.h. on a hot summer day. In such an environment there is no significant accumulation of water, but there is a strong tendency toward chemical degradation of the lubricating oil. This breakdown of the oil results in the formation of acidic materials which in themselves corrode the metal surfaces of the bearings, pistons, etc. Furthermore these acidic products decompose to form hard, carbonaceous deposits which accumulate in the piston ring grooves; still further these acidic products decompose to form also a varnish on the piston skirts and other metal surfaces.

Although, as indicated before, the problems of a crankcase lubricant under such conditions of high temperatures have been dealt with by the use of certain known additives these approaches to the problem have not been entirely satisfactory. Even with the most effective detergents some appreciable deterioration of the lubricating oil still occurs and thus poses a problem.

It is accordingly a principal object of this invention to provide a novel process for the preparation of products which are effective as dispersants in lubricant compositions.

It is another object of this invention to provide novel products which are effective dispersants in lubricant composition intended for use in engines operated at alternating high and low temperatures.

It is another object of this invention to provide novel products which are effective dispersants in lubricant compositions intended for use in engines operated at high speed and therefore at high temperatures.

It is another object of this invention to provide improved lubricant compositions.

These and other objects of the invention are achieved by a lubricating composition consisting essentially of a major proportion of a lubricating oil and

(a) from about 0.1 to about 10 percent by weight of an oil-soluble acylated amine prepared by the process which comprises reacting maleic anhydride with a material selected from the class consisting of aliphatic olefin polymers having an average molecular weight within the range of from about 700 to about 100,000 and chlorinated aliphatic hydrocarbons having an average molecular weight within the range of from about 700 to about 100,000, to form a substituted carboxylic anhydride wherein the substituent group is an aliphatic hydrocarbon radical having at least about 50 aliphatic carbon atoms, mixing a carboxylic acid compound selected from the class consisting of

(1) said substituted carboxylic anhydrides, and  
(2) substituted carboxylic acids corresponding thereto, with at least about one-half an equivalent amount of an alkylene polyamine, and heating the resulting mixture, at a temperature above about 80° C. to effect acylation and remove the water formed thereby, and

(b) from about 0.05 to about 5.0 percent by weight as sulfate ash of an oil-soluble dispersant selected from the class consisting of alkaline earth metal petroleum sulfonates, alkaline earth metal alkyl-aromatic sulfonates, alkaline earth metal alkyl phenates and alkaline earth metal salts of phosphorus acids prepared from polymers of olefins having 2-30 carbon atoms, said polymer having a molecular weight of at least about 750.

It will be seen that the reaction by which component is prepared involves an amidation of a dicarboxylic acid (or anhydride thereof) with a polyamine, and can result in a simple acyclic diamide, a cyclic diamide, a polymeric amide or a combination of any of these types of products. It will be noted also that the amide groups may react fur-

ther to form imide groups and it is believed that a substantial amount of imide formation takes place in the process. Furthermore there is reason to believe that in certain instances there is present in the product an appreciable proportion of amine carboxylic salt.

The size of the substituent of the succinic acid or anhydride is of major importance in the process because it allows the preparation of a product which satisfies the objects of the invention, i.e., one which is effective as a dispersant in the lubricants of this invention. It is critically important that this substituent be large, that it have at least about 50 carbon atoms in its structure. These substituent groups are substantially aliphatic hydrocarbon radicals, including both alkyl and alkenyl radicals. They are commonly derived from polyolefins such as polyethylene, polypropylene, polybutylene, etc., although they may be derived from any substantially aliphatic hydrocarbon.

The substituted succinic acids and anhydrides which are contemplated as a reactant in the process are readily available from the reaction of maleic anhydride with a high molecular weight olefin or a chlorinated high molecular weight olefin. The product from such a reaction is the corresponding alkenyl succinic anhydride. The reaction involves merely heating the two reactants at a temperature of about 150-200° C. The reactions in each case are illustrated by the following equations.



It will be appreciated that the reactions may not go precisely as indicated in the above equations, especially with respect to the particular carbon atom of the olefin or chloride reactant which ultimately becomes attached to the maleic acid or anhydride reactant, but other than this the equations are believed to be illustrative. Furthermore although the product of this reaction has been indicated as being an alkenyl succinic anhydride it is apparent that similar products can be prepared by this process in which the substituent is something other than an alkenyl group. For the purposes of this invention this substituent should, however, be a substantially aliphatic group and in most cases of course it will be an alkyl or alkenyl group. In some cases, it may well be desirable to employ a substituted succinic anhydride in which the substituent is derived for example from a copolymer of styrene and isobutylene, or of a substituted styrene and some other lower aliphatic olefin. In these latter cases the copolymer will be substantially aliphatic, that is, the composition of the copolymer will be predominantly aliphatic, i.e., more than about 80% of the monomeric units will be those of the aliphatic monomer.

As mentioned earlier the size of this substituent group appears to determine the effectiveness of the product of the process of the invention as a dispersant in motor oils. Substituted succinic anhydrides and their derivatives have been known for some time and it has likewise been known that these compounds are useful in lubricants, but their utility heretofore has been predicated upon their rust-preventing properties, corrosion-inhibiting properties, viscosity-temperature characteristics, etc. The usefulness of compositions of this type as dispersants has never been realized and an important aspect of this invention resides in the discovery that by increasing the size of this particular substituents an entirely new property, i.e., dispersancy, can be incorporated into the composition.

The most commonly used sources of these substantially aliphatic hydrocarbon substituents are the polyolefins. These are illustrated by polyethylene, polypropylene, polyisobutylene, etc. A particularly preferred polyolefin

for this use is polyisobutylene. Thus the condensation of a polyisobutylene having a molecular weight of 750 with maleic anhydride yields an alkenyl succinic anhydride which upon further reaction with an ethylene amine produces an especially effective lubricating oil dispersant. Polyisobutylenes of this particular molecular weight are quite economically available and the effectiveness of products prepared from this material makes this starting material particularly desirable for use in a process of this invention.

Other sources of such hydrocarbon substituents are the polymers of higher 1-mono-olefins such as 1-octene, 1-dodecene, and 1-octadecene. These 1-mono-olefins may contain as many as 30 carbon atoms. Interpolymers of these 1-mono-olefins may also be used provided that the interpolymers are substantially aliphatic, and more particularly such interpolymers are preferred in which the composition thereof comprises at least 80%, on a molar basis, of 1-mono-olefin units.

Interpolymers of such 1-mono-olefins with isoprene, butadiene, piperylene, vinyl cyclohexene, chloroprene, vinyl chloride, styrene, vinyl acetate, chlorostyrene, and vinyl alkyl ethers are thus contemplated.

The molecular weight of the substantially aliphatic hydrocarbon substituent of component (a) may range from one having the minimum of about 50 carbon atoms or a molecular weight of about 700 up to one having a molecular weight of 75,000 or 100,000 or even higher. It should be noted that the expression "hydrocarbon substituent," as is used in the specification and claims, denotes a substituent which is hydrocarbon or substantially hydrocarbon in character. Thus, the substituent may contain polar groups provided, however, that such polar groups are not present in proportions sufficiently large to alter significantly the hydrocarbon character of the substituent. The polar groups which may be present are exemplified by chloro, bromo, iodo, keto, aldehydo, ether and nitro radicals. The maximum proportion of such polar groups in the substituent is approximately 10 percent based upon the weight of the hydrocarbon portion of the substituent.

The substituted succinic anhydride ordinarily is reacted directly with the alkylene amine although in some circumstances it may be desirable first to convert the anhydride to the acid before reaction with the amine. In other circumstances it may be desirable to prepare the substituted succinic acid by some other means and to use an acid prepared by such other means in the process. In any event either the acid or the anhydride may be used in the process of this invention.

The term "alkylene amine" is used in a generic sense to denote a class of polyamines conforming for the most part to the structure



in which  $x$  is an integer and R is a low molecular weight alkyl radical or hydrogen. Thus it includes for example ethylene diamine, diethylene triamine, triethylene tetramine, tetraethylene pentamine, pentaethylene hexamine, etc. These compounds are discussed in some detail under the heading, "Ethylene Amines," in "Encyclopedia of Chemical Technology," Kirk and Othmer, vol. 5, pages 898-905, Interscience Publishers, New York (1950). Such compounds are prepared most conveniently by the reaction of ethylene or propylene dichloride with ammonia. This process results in the production of somewhat complex mixtures of ethylene amines including cyclic condensation products such as piperazines and these mixtures find use in the process of this invention. On the other hand quite satisfactory products may be obtained also by the use of pure ethylene amines. An especially useful ethylene amine, for reasons of economy as well as effectiveness as a dispersant, is a mixture of ethylene amines prepared by the reaction of ethylene chloride and ammonia, having a composition which cor-

responds to that of a tetraethylene pentamine. This is available in the trade under the trade name "Polyamine H."

Other polyamines quite suitable for the purposes of this invention, include alkylene polyamines such as 1,3-propylene diamine, 1,4-butylene diamine, propylene polyamines in which the amino groups are attached to the 1- and 3-carbon atoms, butylene polyamines in which the amino groups are attached to the 1- and 4-carbon atoms, and the C-alkyl-substituted derivatives of these and other such alkylene polyamines. For the most part, polyalkylene polyamines having up to about 10 alkylene groups and up to about 10 carbon atoms in each alkylene group are useful.

It has been noted that at least one-half of a chemical equivalent amount of the alkylene amine per equivalent of substituted succinic anhydride must be used in the process to produce a satisfactory product with respect to dispersant properties and generally it is preferred to use these reactants in equivalent amounts. Amounts up to 2.0 chemical equivalents (per equivalent of substituted succinic anhydride) have been used with success, although there appears to be no advantage attendant upon the use of more than this amount. The chemical "equivelency" of the alkylene amine reaction is based upon the nitrogen content, i.e., one having four nitrogens per molecule has four equivalents per mole.

The reaction of the process involves a splitting out of water and the reaction conditions are such that this water is removed as it is formed. Presumably the first principal reaction that occurs, following salt formation, is the formation of a half amide



followed then by salt formation



and involving finally dehydration of this salt to form the product



The first two of these reactions appear to take place spontaneously (when a substituted succinic anhydride is used) upon mixing, but the third requires heating. Temperatures within the range of about 80° C. to about 200° C. are satisfactory, and within this range it is preferred to use a reaction temperature of from about 100° C. to about 160° C. A useful method of carrying out this step is to add some toluene to the reaction mixture and to remove the water by azeotropic distillation. As indicated before there is also some imide-formation.

Component (a) is unique in that it acts as a dispersant in lubricant compositions although it contains no metal within its molecular structure. Component (b) on the other hand may be any of several well-known dispersants all of which are metal salts. As indicated earlier these well-known dispersants are the alkaline earth metal sulfonates, the alkaline earth metal alkyl phenates and the alkaline earth metal salts of phosphorus acids prepared from polymers of olefins having 2-4 carbon atoms.

Of the alkaline earth metal salts contemplated for use in the lubricants of this invention the barium and calcium salts find widest applicability. The magnesium and strontium salts have been used somewhat, but on a much smaller scale than the barium and calcium salts. All, however, are useful for the purposes of this invention and all are contemplated as being within the scope thereof.

The sulfonates include chiefly those sulfonates derived from petroleum. These are the mahogany sulfonates prepared by sulfonation of naphthenic stocks with con-

centrated sulfuric acid, oleum or sulfur trioxide, etc., as well as those derived from the chlorosulfonation, with chlorine and sulfur dioxide, of substantially aliphatic petroleum fractions. These chlorosulfonated aliphatic fractions are saponified with sodium hydroxide and then converted to the alkaline earth metal salt by double decomposition with the metal chloride. A variety of such sulfonation processes are available and the oil soluble sulfonates derivable from any of these are suitable for use in this invention. The synthetic sulfonates prepared by sulfonation of alkylated aromatic hydrocarbons likewise are valuable for this purpose. A common sulfonate of this type is that prepared by the sulfonation of a dodeceny1 benzene prepared from tetrapropylene and benzene.

15 The alkaline earth metal alkyl phenates include those derived from such simple alkyl phenols as heptylphenol, octylphenol, decylphenol, etc., and also condensation products prepared from such alkyl phenols and from 0.5 to 2.0 moles of formaldehyde or acetaldehyde. The 20 alkyl phenate may be derived also from alkyl phenol sulfides such as for example the reaction product of 1 mole of sulfur monochloride with 2 moles of diisobutyl phenol.

25 The phosphorus acids from which component (b) may be derived include several types of acidic materials. They 30 are prepared in most instances from polyisobutylene, although they may be prepared from any substantially aliphatic polymer within the limits of the definition of component (b). Thus, the polymer may be a polyethylene, polypropylene, polyhexene, polydodecene, or a polymer of other 1-mono-olefins having as many as 30 carbon atoms. It may likewise be an interpolymer in which the 35 preponderant proportion of monomeric units is derived either from ethylene, propylene, isobutylene, or any other 1-mono-olefin having up to 30 carbon atoms. Such interpolymers are illustrated by an interpolymer of 95 molar parts of isobutylene and 5 molar parts of styrene.

In general those interpolymers are preferred in which 40 at least 80%, on a molar basis of the interpolymer composition is derived from the aliphatic 1-mono-olefin. 45 Such preferred interpolymers may include up to about 20%, on a molar basis, of units derived from isoprene, butadiene, piperylene, vinyl cyclohexene, chloroprene, vinyl chloride, styrene, vinyl acetate, chlorostyrene, or a vinyl alkyl ether. The proportion of 1-mono-olefin units present in such interpolymers influences the oil solubility of the phosphorus acid salt derived from any particular interpolymer.

The molecular weight of this lower olefin polymer 50 reactant to be employed in the preparation of component (b) may vary within a rather wide range. Thus, it may be as low as about 750 or, on the other hand, range upward to as high as 75,000 or, in some instances, even higher. The various types of phosphorus acids available 55 from these polymers are prepared by reaction of the polymers with any of several well-known phosphorizing agents, followed by reaction with a reagent having an active hydrogen atom, usually water, and then neutralization with a basic, metal neutralizing compound such as barium oxide or lime.

60 Illustrative phosphorus acids include, for example, the reaction products of any of these polymers with phosphorus pentasulfide and sulfur, followed by steam treatment and then neutralization with a basic inorganic alkaline earth metal compound, such as barium oxide. Alternatively the neutralization step may be effected prior to the step of steam treatment. Another important type of phosphorus acid is that prepared from a polyolefin as defined in component (b) with phosphorus trichloride and sulfur followed by the neutralization and steam-treatment steps. Still another such phosphorus acid is that which can be prepared by the chlorination of the polyolefin followed by reaction with phosphorus trichloride and either steam or an alkyl phenol. This acid then, of course, can be neutralized with a basic metal compound. 75 Another type of phosphorus acid is that which is prepared

by the reaction of an aliphatic polyolefin with phosphorus and sulfur monochloride, followed by steam treatment and neutralization. Still another type of phosphorus acid can be prepared by reaction of a polymer of the type described before with a phosphorus sulfide, followed by steam treatment and neutralization with a basic inorganic alkaline earth metal compound.

A general definition of the phosphorus acid salts contemplated for use as component (b) includes those prepared by reaction of a polymer of a 1-mono-olefin with a phosphorizing agent, followed by treatment of the resulting product with a hydrolyzing agent and neutralizing agent. The phosphorizing agents include phosphorus sulfides, phosphorus chlorides, thiophosphoryl chloride, phosphorus pentoxide, phosphorus, and combinations of these with sulfurizing agents such as sulfur, sulfur chloride, and sulfur monochloride. Illustrative combinations of these phosphorizing and sulfurizing agents include phosphorus pentasulfide and sulfur monochloride, phosphorus and sulfur monochloride, and phosphorus pentachloride and sulfur.

The structure of such phosphorus acids is not known and in fact it is commonly believed that an acid prepared in this fashion, viz., by reaction of a polyolefin with a phosphorizing agent followed by hydrolysis of the intermediate phosphorized product, is really a mixture, not only of two or more different acids, but a mixture perhaps of different types of acids. Thus, this mixture may contain acids having carbon-to-phosphorus bonds or acids having carbon-to-oxygen-to-phosphorus bonds, or carbon-to-sulfur-to-phosphorus bonds. Inasmuch, however, as the structure of these phosphorus acids is not known, it is necessary to refer to them in terms of the process by which they can be prepared.

The basicity of any of these alkaline earth metal detergents can be varied considerably. Starting with the free acid, it may be neutralized to provide merely the normal alkaline earth metal salt which is useful, or it can be treated with an excess of the neutralizing alkaline earth metal compound to form a basic salt. This also, of course, is useful. Generally speaking, however, it is preferred to neutralize the acid with a considerable excess of basic inorganic alkaline earth metal compound and to carbonate the product so that that product contains a stoichiometrically excessive amount of metal with respect to the organic acidic anions present in the product. Various promoters may be used to assist in the incorporation of such excessive metal and these include principally phenolic compounds and low molecular weight alcohols.

Yet another type of alkaline earth metal salt may be prepared. Using as a starting material the metal salt of any of the organic acids of component (b), such metal salt may be sulfonated with chlorosulfonic acid to yield an acidic metal salt. This acidic metal salt then may be neutralized with a basic inorganic alkaline earth metal compound to form either a normal or a basic alkaline earth metal salt. This process is described in more detail in copending application Ser. No. 658,737 and the details of the disclosure of this copending application are incorporated herein by reference. Thus a sodium mahogany sulfonate may be sulfonated with chlorosulfonic acid and then treated with a stoichiometric excess of barium oxide in the presence of methanol, carbonated and then filtered to yield an especially effective additive for use in the combination of this invention. Another very good additive for such use can be prepared by the reaction of polyisobutylene having a molecular weight of about 750 with phosphorus trichloride and sulfur, followed by treatment with steam, then neutralization with barium oxide to form the normal barium salt, followed by sulfonation with chlorosulfonic acid and neutralization with a stoichiometric excess of barium oxide in the presence of heptylphenol, carbonation and filtration. Similarly the sulfonation of a neutralized chlorinated polyisobutylene (M.W.:850)-phosphorus trichloride-steam product is an

excellent starting material for the preparation of satisfactory components in the combination of this invention.

The combination of additives of this invention have been found to be effective in many different types of lubricating oils. Oils derived from paraffinic and asphaltic crudes are benefitted thereby as well as all of the ordinarily available synthetic lubricants. These latter include the polyethers, polyesters, silicones, voltolized oils, etc.

*Example 1.*—A polyisobutylene succinic anhydride was prepared by the reaction of a chlorinated polyisobutylene with maleic anhydride at 200° C. The polyisobutylene radical had an average molecular weight of 850 and the resulting alkenyl succinic anhydride was found to have an acid number of 113 (corresponding to an equivalent weight of 500). To a mixture of 500 grams (1 equivalent) of this polyisobutylene succinic anhydride and 160 grams of toluene there was added at room temperature 35 grams (1 equivalent) of diethylene triamine. The addition was made portionwise throughout a period of 15 minutes, and an initial exothermic reaction caused the temperature to rise to 50° C. The mixture then was heated and a water-toluene azeotrope distilled from the mixture. When no more water would distill the mixture was heated to 150° C. at reduced pressure to remove the toluene. The residue was diluted with 350 grams of mineral oil and this solution was found to have a nitrogen content of 1.6%.

*Example 2.*—The procedure of Example 1 was repeated using 31 grams (1 equivalent) of ethylene diamine as the amine reactant. The nitrogen content of the resulting product was 1.4%.

*Example 3.*—The procedure of Example 1 was repeated using 55.5 grams (1.5 equivalents) of an ethylene amine mixture having a composition corresponding to that of triethylene tetramine. The resulting product had a nitrogen content of 1.9%.

*Example 4.*—The procedure of Example 1 was repeated using 55.0 grams (1.5 equivalents) of triethylene tetramine as the amine reactant. The resulting product had a nitrogen content of 2.5%.

*Example 5.*—To a mixture of 140 grams of toluene and 400 grams (0.78 equivalent) of a polyisobutylene succinic anhydride (having an acid number of 109 and prepared from maleic anhydride and the chlorinated polyisobutylene of Example 1) there was added at room temperature 63.6 grams (1.55 equivalents) of an ethylene amine mixture having an average composition corresponding to that of tetraethylene pentamine and available from carbide and carbon under the trade name, "Polyamine H." The mixture was heated to distill the water-toluene azeotrope and then to 150° C. at reduced pressure to remove the remaining toluene. The residual polyamide had a nitrogen content of 4.7%.

*Example 6.*—The procedure of Example 1 was repeated using 46 grams (1.5 equivalents) of ethylene diamine as the amine reactant. The product which resulted had a nitrogen content of 1.5%.

*Example 7.*—A polyisobutylene succinic anhydride having an acid number of 105 and an equivalent weight of 540 was prepared by the reaction of a chlorinated polyisobutylene (having an average molecular weight of 1,050 and a chlorine content of 4.3%) and maleic anhydride. To a mixture of 300 parts by weight of the polyisobutylene succinic anhydride and 160 parts by weight of mineral oil there was added at 65–95° C. an equivalent amount (25 parts by weight) of Polyamine H (identified in Example 5). This mixture then was heated to 150° C. to distill all of the water formed in the reaction. Nitrogen was bubbled through the mixture at this temperature to insure removal of the last traces of water. The residue was diluted by 79 parts by weight of mineral oil and this oil solution found to have a nitrogen content of 1.6%.

*Example 8.*—A mixture of 2,112 grams (3.9 equivalents) of the polyisobutylene succinic anhydride of Example 7, 136 grams (3.9 equivalents) of diethylene tri-

amine, and 1060 grams of mineral oil was heated at 140-150° C. for one hour. Nitrogen was bubbled through the mixture at this temperature for four more hours to aid in the removal of water. The residue was diluted with 420 grams of mineral oil and this oil solution was found to have a nitrogen content of 1.3%.

*Example 9.*—To a solution of 1,000 grams (1.87 equivalents) of the polyisobutenyl succinic anhydride of Example 7, in 500 grams of mineral oil there was added at 85-95° C. 70 grams (1.87 equivalents) of tetraethylene pentamine. The mixture then was heated at 150-165° C. for four hours, blowing with nitrogen to aid in the removal of water. The residue was diluted with 200 grams of mineral oil and the oil solution found to have a nitrogen content of 1.4%.

*Example 10.*—A polypropenyl succinic anhydride was prepared by the reaction of a chlorinated polypropylene (having a molecular weight of about 900 and a chlorine content of 4%) and maleic anhydride at 200° C. The product had an acid number of 75. To a mixture of 390 grams (0.52 equivalent) of this polypropenyl succinic anhydride, 500 grams of toluene, and 170 grams of mineral oil there was added portionwise 22 grams (0.52 equivalent) of Polyamine H. The reaction mixture was heated at reflux temperature for three hours and water removed from an azeotrope with toluene. The toluene then was removed by heating to 150° C./20 millimeters. The residue was found to contain 1.3% of nitrogen.

*Example 11.*—A substituted succinic anhydride was prepared by reacting maleic anhydride with a chlorinated copolymer of isobutylene and styrene. The copolymer consisted of 94 parts by weight of isobutylene units and 6 parts by weight of styrene units, had an average molecular weight of 1,200, and was chlorinated to a chlorine content of 2.8% by weight. The resulting substituted succinic anhydride had an acid number of 40. To 30 710 grams (0.51 equivalent) of this substituted succinic anhydride and 500 grams of toluene there was added portionwise 22 grams (0.51 equivalent) of Polyamine H. The mixture was heated at reflux temperature for three hours to remove by azeotropic distillation all of the water formed in the reaction, and then at 150° C./20 millimeters to remove the toluene. The residue contained 1.1% by weight of nitrogen.

*Example 12.*—A substituted succinic anhydride was prepared by reacting maleic anhydride with a chlorinated copolymer of isobutylene and isoprene. The copolymer consisted of 99 parts of isobutylene units and 1% by weight of isoprene units. The molecular weight of the copolymer was 28,000 and the chlorine alkenyl succinic anhydride had an acid number of 54. A stirred mixture of 228 grams (0.22 equivalent) of an oil solution of this alkenyl succinic anhydride, 58 grams of additional mineral oil, 500 grams of toluene and 9.3 grams (0.22 equivalent) of Polyamine H was heated at 110-120° C. for three hours, water being removed from an azeotrope with toluene. When all of the water had thus been removed the toluene was distilled by heating to 150° C./20 millimeters. The residue was found to have a nitrogen content of 1.1%.

*Example 13.*—A polyisobutenyl succinic anhydride was prepared by the reaction of a chlorinated polyisobutylene with maleic anhydride. The chlorinated polyisobutylene had a chlorine content of 2% and an average molecular weight of 11,000. The polyisobutenyl succinic anhydride had an acid number of 48. A mixture of 410 grams (0.35 equivalent) of this anhydride, 15 grams (0.35 equivalent) of Polyamine H and 500 grams of toluene was heated at reflux temperature for four hours to remove water from an azeotrope with toluene. The toluene then was removed by heating to 150° C./20 millimeters. The nitrogen content of the residue was 1.3%.

*Example 14.*—The procedure for Example 5 was repeated except that 0.94 equivalent of Polyamine H was

used instead of 1.55 equivalents. The nitrogen content of the product was 3%.

*Example 15.*—A polyisobutenyl-substituted succinic acid was prepared by hydrolysis of the corresponding anhydride (prepared in turn by the condensation of a chlorinated polyisobutylene and maleic anhydride). To 1152 grams (1.5 equivalents) of a 70% mineral oil solution of this polyisobutenyl succinic acid having an acid number of 62 there was added at room temperature 59.5 grams (1.5 equivalents) of Polyamine H. This mixture was heated at 150-167° C. for 7 hours during which time a total of 19.5 grams of water was distilled from the mixture. The residue was diluted with 174 grams of mineral oil and then filtered at 150° C. The filtrate had a nitrogen content of 1.6%.

*Example 16.*—A mixture of 1056 grams (2.0 equivalents) of the polyisobutenyl succinic anhydride of the preceding example (in which the polyisobutenyl group has a molecular weight of 850), 89 grams (2.0 equivalents) of dis-(1,2-propylene) triamine (having a nitrogen content of 31.3%), 370 grams of mineral oil and 100 grams of toluene was heated at reflux temperature (180-190° C.) for 5 hours. A total of 18 grams of water was collected from the water-toluene azeotrope. The residue was heated to 150° C./20 mm. to remove any last traces of water which might have remained. The nitrogen analysis of this residue was 1.9%.

*Example 17.*—A polyisobutylene having an average molecular weight of 50,000 was chlorinated to a chlorine content of 10% by weight. This chlorinated polyisobutylene was reacted with maleic anhydride to produce the corresponding polyisobutenyl succinic anhydride having an acid number of 24. To 6,000 grams (2.5 equivalents) of this anhydride there was added portionwise at 35 70-105° C. 108 grams (2.55 equivalents) of Polyamine H over a period of 45 minutes. The resulting mixture was heated for four hours at 160-180° C. while nitrogen was bubbled throughout to remove water. When all of the water had been removed the product was filtered and the filtrate found to have a nitrogen content of 0.6%.

*Example 18.*—A mixture of 1,000 grams (1.89 equivalents) of a polyisobutenyl succinic anhydride in which the polyisobutenyl group has an average molecular weight of 850, 60 grams (1.45 equivalents) of an ethylene amine mixture having a nitrogen content of 33.9%, 15 grams (0.44 equivalent) of diethylene triamine, and 161 grams of toluene was heated at 12-174° C. (reflux temperature) for 9 hours. A total of 17 ml. of water was removed from the toluene-water azeotrope. The residual product was found to have a nitrogen analysis of 1.4%.

*Example 19.*—

(a) A mixture of 2,500 parts (3.0 equivalents) of polyisobutylene having an average molecular weight of 840 and 84 parts (as a catalyst) of a 40% oil solution of a barium dialkyl phosphorodithioate (in which the alkyl radicals are 50% octyl, 12% cyclohexyl and 38% hexyl) was heated to 245° F. To this mixture there was added 133 parts (4.0 equivalents) of sulfur and the mixture heated to 310° F. Then 458 parts (3.3 equivalents) of phosphorus trichloride was introduced beneath the surface of the reaction mixture over a period of 4 hours. The temperature was maintained at 310-320° F. throughout and after an additional 30 minutes of heating at this temperature and the reaction mixture was heated at reduced pressure to remove any volatile components. The residue was blown with steam for four hours at 320-330° F., then dried with nitrogen to a water content of less than 0.25%. The acidic product had a neutralization number of 68.

(b) To a mixture of 2,090 parts of mineral oil and 250 parts of water at 180° F. there was added 70 parts (0.9 equivalent) of barium oxide and then 1,900 parts (2.3 equivalents) of the above acid. The latter was added throughout a period of 1.5 hours and during this time and throughout an additional 1.5 hours there was

added 1,337 parts (17.4 equivalents) more of barium oxide. The addition of barium oxide caused the temperature to rise to 270° F. and when all of the barium oxide has been added 443 parts (2.3 equivalents) of heptyl phenol was added. This mixture was dehydrated by heating at 300° F. for two hours and blowing with nitrogen. Thereupon carbon dioxide was blown through the solution for 5 hours at 280° F. The thus carbonated mixture was diluted with 1,200 parts of mineral oil and filtered through a siliceous filter aid. The filtrate showed the presence of 26.0% barium as sulfate ash.

*Example 20.*—An acid was prepared by the process of Example 19(a) using a polyisobutylene having an average molecular weight of 41,000. This acid (300 parts, 0.12 equivalent) was added over a 1.3 hour period to a mixture of 120 parts of mineral oil, 15 parts of water, and 5 parts (0.06 equivalent) of barium oxide. Throughout this period and an additional 1.3 hours 77 parts (1.0 equivalent) of barium oxide was added to the mixture. Then the mixture was heated to 240° F. and 38 parts (0.2 equivalent) of heptyl phenol was added throughout a period of 30 minutes. The temperature was increased to 300° F., nitrogen bubbled through for an hour, and then carbon dioxide for 10 hours. Forty parts of a siliceous filter aid was added and the mixture filtered. The filtrate showed a barium content of 14.5% as sulfate ash.

*Example 21.*—An acid was prepared by the process of Example 19(a) except that the polyisobutylene had an average molecular weight of 44,000. To a mixture of 392 parts of mineral oil, 15 parts of water and 22 parts (0.3 equivalent) of barium oxide there was added at 180° F. over a period of 2.7 hours, 292 parts (0.23 equivalent) of this acid. After heating for an additional 90 minutes, 7 parts more (0.1 equivalent) of barium oxide was added. This mixture then was heated to 300° F., blown with nitrogen for 30 minutes and filtered through a siliceous filter aid. The filtrate had a barium content of 2.5% as sulfate ash.

*Example 22.*—

(a) Polyisobutylene having an average molecular weight of 1,000 was chlorinated to a chlorine content of 4.3%.

(b) To 900 parts (1.0 equivalent) of this chlorinated polyisobutylene at 230–370° F. there was added portionwise over a period of 15 hours 150 parts (1.1 equivalent) of phosphorus trichloride. After an additional 2 hours of heating at 390° F. the mixture was freed of volatile components by heating at reduced pressure for an additional 1.5 hours and then blowing with nitrogen for 2 hours. Steam at 320–330° F. was blown through the mixture for 4 hours at which point successive samples showed no change in neutralization number.

To a mixture of 495 parts of mineral oil, 100 parts (0.5 equivalent) of heptyl phenol, 38 parts of water and 62 parts (0.8 equivalent) of barium oxide at 180–200° F. there was added over a period of 3 hours 400 parts (0.2 equivalent) of the above acid. An additional 257 parts (3.3 equivalents) of barium oxide was added to the mixture whereupon carbon dioxide was bubbled through for 3 hours at 270–280° F. The mixture was diluted with 281 parts of mineral oil and then filtered through a siliceous filter aid. The filtrate had a barium content of 25.0% as sulfate ash.

*Example 23.*—

(a) To 783 parts (0.87 equivalent) of the chlorinated polyisobutylene of Example 22(a) there was added at 210° F. 125 parts (0.9 equivalent) of phosphorus trichloride. Heptyl phenol (205 parts, 1.0 equivalent) then was added portionwise over a period of 2 hours. The temperature was maintained at about 180° F. for an additional 3 hours and then increased to 375° F. and held there for another 2 hours. Nitrogen was blown through the mixture for 30 minutes and then steam at 350–380° F. until the neutralization number leveled off at about 50.

(b) To a mixture of 700 parts of mineral oil, 18 parts of water and 27 parts (0.35 equivalent) of barium oxide at 180° F. there was added 171 parts (0.15 equivalent) of the above acid. Eleven parts (0.06 equivalent) of heptyl phenol was added and the mixture heated for an additional hour at 190° F. Then 113 parts (1.47 equivalents) more of barium oxide was added. After another hour of heating, carbon dioxide was blown through the mixture for 6 hours and then nitrogen for 30 minutes. The mixture was diluted with 118 parts of mineral oil and filtered through a siliceous filter aid. The filtrate showed a barium content of 26.5% as sulfate ash.

*Example 24.*—The process of Example 23 was repeated except that 1.5 moles of phosphorus trichloride and 0.3 mole of heptyl phenol was used in the preparation of the acid of (a). Also the temperature of steam blowing was reduced to 310° F. The product had a barium content of 26.5% as sulfate ash.

*Example 25.*—To a mixture of 6,640 grams (13.3 equivalents) of barium petroleum sulfonate, 873 grams (4.5 equivalents) of heptyl phenol and 2,200 grams of water in 8,500 grams of mineral oil there was added at 180–300° F. 4,000 grams (52.2 equivalents) of barium oxide. The stirred reaction mixture then was heated to 300° F. to remove the water and carbon dioxide was blown through the mixture at this temperature until it was neutral. The product was diluted with 4,169 grams of mineral oil and filtered through a siliceous filter aid. The filtrate was further diluted until the barium content was 25% as sulfate ash.

*Example 26.*—To a mixture of 6,245 grams (12.5 equivalents) of barium petroleum sulfonate, 1,460 grams (7.5 equivalents) of heptyl phenol, and 2,100 grams of water in 8,045 grams of mineral oil there was added at 180° F. 7,400 grams (96.5 equivalents) of barium oxide. The addition of barium oxide caused the temperature to rise to 290° F. which temperature was maintained until all of the water had been distilled away. The mixture then was blown with carbon dioxide until it was substantially neutral. 5,695 grams of mineral oil was added and the mixture filtered through a siliceous filter aid. The filtrate was diluted further with mineral oil to a barium content of 30.5% as sulfate ash.

*Example 27.*—The barium salt of a phosphorus- and sulfur-containing acid was prepared by reaction of polyisobutylene (M.W.:850) with phosphorus pentasulfide and sulfur followed by treatment with steam and neutralization with barium oxide. To 5,850 grams (6.8 equivalents) of this barium salt there was added portionwise at 120–160° F. over a period of 2 hours 419 grams (3.6 equivalents) of chlorosulfonic acid. The mixture then was blown with nitrogen to remove gaseous materials.

To the resulting sulfonic acid and 858 grams (4.4 equivalents) of heptyl phenol there was added a slurry of 400 grams (5.2 equivalents) of barium oxide and 71 grams of water in 3,300 grams of mineral oil. After this mixture had been agitated at 150–220° F. for 30 minutes an additional 1,931 grams (25.2 equivalents) of barium oxide was added. Enough water was introduced, either as steam or liquid water to hydrate all of the barium oxide. At a temperature of 270° F. carbon dioxide was bubbled through the mixture until it was substantially neutral. The mixture then was filtered through a siliceous filter aid to yield a filtrate which was further diluted with mineral oil to a barium content of 25.0% as sulfate ash.

*Example 28.*—To a mixture of 1,000 parts (1.0 equivalent) of sodium petroleum sulfonate, a solution of 69.5 parts weight (1.2 equivalents) of 96% calcium chloride in 84 parts of water there was added at 200° F. over a 2-hour period 72 parts (1.7 equivalents) of 85% calcium hydroxide. This mixture was heated for an additional 2 hours at 200° F. and then cooled to 120° F. while adding 130 parts of methanol. Carbon dioxide was bubbled through the mixture at this temperature until it was substantially neutral and then the temperature was

raised to 300° F. to remove the methanol and water. The mixture was filtered through a siliceous filter aid to yield a clear filtrate as the product. It had a calcium content of 16.4% as sulfate ash.

*Example 29.*—A slurry of 1,854 grams (9.0 equivalents) of diisobutyl phenol, 370 grams (10.0 equivalents) of calcium hydroxide, 450 grams of water and 4,800 grams of oil was prepared and heated to 75° C. To this slurry there was added 90 ml. of ammonium hydroxide and 405 grams (13.5 equivalents) of paraformaldehyde. This mixture was stirred to reflux temperature for 1 hour and then dried by heating to 150° C. The mixture was filtered through a siliceous filter aid to yield a filtrate having a calcium content of 7.0% as sulfate ash.

*Example 30.*—A mixture of 1,000 grams (1.05 equivalents) of polyisobutylene, 37 grams (1.2 equivalents) of yellow phosphorus, 157 grams (1.2 equivalents) of sulfur monochloride and 1,000 grams of mineral oil was heated at 160° C. for 6 hours in an atmosphere of nitrogen. The reaction mixture then was blown with steam at this same temperature for 2 hours. To this steam-treated mixture there was added 198 grams (2.6 equivalents) of barium oxide and 187 grams of water. The resulting mixture was heated at 150° C. for an hour and then filtered through a siliceous filter aid. This filtrate was heated at 150° C. with 393 grams (5.1 equivalents) of barium oxide and 168 grams (0.88 equivalent) of heptyl phenol, then carbonated with carbon dioxide until it was neutral. Filtration yielded a clear product having a barium content of 21.7.

*Example 31.*—To a solution of 47 parts of polyisobutylene having an average molecular weight of 60,000, in 76 parts of mineral oil, heated at 200° F., there was added 2.8 parts of phosphorous pentasulfide. This mixture was heated at 500° F. for two hours, then cooled to 300° F. Steam was blown through the mixture at this temperature (for 6 hours) until the acid number of the mixture increased no further.

To 40 parts of this acid, having an acid number of 12.0, there was added 3.3 parts of barium oxide and the slurry was heated to 265° F. The neutralized mixture was diluted with 79 parts of mineral oil and then filtered. The filtrate was found to have a sulfate ash content of 1.7%.

*Example 32.*—An alkenyl succinic anhydride was prepared by chlorination of a polyisobutylene having an average molecular weight of 900, followed by reaction of this chlorinated product with maleic anhydride. To 265 parts of this polyisobutylene succinic anhydride there was added 58 parts of heptyl phenol, 1,527 parts of mineral oil and 55 parts of water. This mixture was heated to 70° C. whereupon 460 parts of barium oxide was added. The temperature was increased to 150° C. and carbon dioxide blown through the mixture until it was slightly acidic. The carbonated mixture was filtered to yield a filtrate having a sulfate ash content of 23.3%.

In the preceding examples all parts are by weight.

The dispersant qualities of the combination of the additives prepared by the processes of the above-illustrated examples are most striking when they are used in mineral oil lubricants. These products are miscible in such lubricants in all proportions, and normally the acylated amine product is employed in a concentration ranging from 0.1 to about 10.0% by weight of the lubricant composition whereas the alkaline earth metal-containing dispersant is employed in a concentration within the range of from about 0.05 to about 5.0% by weight as sulfate ash of the lubricant composition. The optimum concentration of each additive depends largely upon the nature of the particular base mineral oil stock and types of service to which the lubricants are to be subjected. In the case of the acylated amine additive this optimum concentration is within the narrower range of from about 0.5% to about 3%. For the alkaline earth metal-containing dispersant this narrower optimum range is from about 0.05 to about 2% by weight as sulfate ash.

As indicated earlier, the combination of additives of this invention may be used with advantage in synthetic lubricants also.

The lubricating compositions of this invention are effective for use in the crankcases of the internal combustion engines employed either under conditions of continuous high speed and high temperatures as well as under conditions of stop-and-go driving, idling, low speed, etc.

The efficacy of these lubricant compositions under conditions of high speed, high temperature operation is shown by the results of engine tests carried out in accordance with U.S. Army Ordnance tentative specification AXS-1551. This test is known as the Caterpillar CRC-L-1 engine test and the particular test to which the lubricants of this invention were subjected is a modification of that test, the modification consisting of the use of a fuel having a sulfur content of 1% (significantly higher than that of the specified fuel). The results of such tests carried out on lubricants of this invention as well as lubricants containing only one of the two types of dispersants are shown as follows.

| Lubri-<br>cant | Additives                                                                                                                | Time<br>(hrs.) | Ring<br>Filling,<br>percent | Piston<br>Cleanli-<br>ness |
|----------------|--------------------------------------------------------------------------------------------------------------------------|----------------|-----------------------------|----------------------------|
| 1.....         | 0.9% of a product prepared as in Example 7 except that the polyisobutylene radical contains an average of 61 carbons.    | 480            | 6                           | 99.0                       |
| 30.....        | 1.75% of the product of Example 20.                                                                                      | 240            | 1                           | 89.0                       |
| 2.....         | 1.4% of a product prepared as in Example 7 except that the polyisobutylene radical contains an average of 61 carbons.    | 360            | 39                          | 95.5                       |
| 3.....         | 1.9% of the product of Example 20.                                                                                       | 240            | 11                          | 92.0                       |
| 4.....         | 0.66% of a product prepared as in Example 7 except that toluene was used as the solvent.                                 | 120            | 1                           | 89.0                       |
| 5.....         | 0.57% of the product of Example 19.                                                                                      | 240            | 47                          | 81.0                       |
| 6.....         | 0.3% of the product of Example 19.                                                                                       | 240            | 11                          | 95.5                       |
| 7.....         | 0.71% of the product of Example 14.                                                                                      | 480            | 23                          | 95.5                       |
| 8.....         | 0.3% of the product of Example 19.                                                                                       | 240            | 5                           | 93.5                       |
| 9.....         | 0.81% of the product prepared as in Example 7 except that the polyisobutylene radical contains an average of 61 carbons. | 240            | 1                           | 94.5                       |
| 10.....        | 0.3% of the product of Example 23.                                                                                       | 480            | 26                          | 88.0                       |
| 11.....        | 0.1% of the product of Example 23.                                                                                       | 480            | 2                           | 93.0                       |
| 12.....        | 0.54% of the product of Example 23.                                                                                      | 360            | 30                          | 94.0                       |
| 13.....        | 0.02% of the product prepared as in Example 7 except that the polyisobutylene radical contains an average of 61 carbons. | 480            | 18                          | 95.5                       |
| 14.....        | 0.2% of the product of Example 22.                                                                                       | 480            | 24                          | 94.0                       |
| 15.....        | 0.53% of the product of Example 22.                                                                                      | 480            | 8                           | 90.0                       |
| 16.....        | 0.1% of the product prepared as in Example 7 except that the polyisobutylene radical contains an average of 61 carbons.  | 240            | 17                          | 97.5                       |
| 17.....        | 0.02% of the product of Example 24.                                                                                      | 480            | 18                          | 95.5                       |
| 18.....        | 0.57% of the product of Example 24.                                                                                      | 480            | 22                          |                            |
| 75.....        | 1.08% of the product of Example 18.                                                                                      |                |                             |                            |
|                | 0.2% of the product of Example 22.                                                                                       |                |                             |                            |

| Lubri-cant | Additives                                                                                                                                                                                                                                                                     | Time (hrs.) | Ring Filling, percent | Piston Cleanli-ness |
|------------|-------------------------------------------------------------------------------------------------------------------------------------------------------------------------------------------------------------------------------------------------------------------------------|-------------|-----------------------|---------------------|
| 19         | 0.52% of the product of Example 7.<br>0.57% of a product prepared as in Example 25 except that the barium sulfonate was a mixture of 90 parts of barium petroleum sulfonate and 10 parts of barium alkaryl sulfonate.                                                         | 480         | 7                     | 95.5                |
| 20         | 0.62% of a product prepared as in Example 25 except that the barium sulfonate was a mixture of 90% barium petroleum sulfonate and 10% barium alkaryl sulfonate.                                                                                                               | 120         | 3.4                   | 90.1                |
| 21         | 0.52% of the product of Example 7.<br>0.27% of the product of Example 26.<br>0.17% of the barium salt of a phosphorus-and-sulfur-containing acid prepared by reaction of polyisobutylene (M.W.:350) with phosphorus pentasulfide and sulfur followed by treatment with steam. | 120         | 1                     | 96.5                |
| 22         | 0.30% of the product of Example 26.<br>0.19% of the barium salt of a phosphorus-and-sulfur-containing acid prepared by reaction of polyisobutylene (M.W.:350) with phosphorus pentasulfide and sulfur followed by treatment with steam.                                       | 120         | 11                    | 84.5                |
| 23         | 1.35% of the product of Example 7.<br>0.3% of the product of Example 31.                                                                                                                                                                                                      | 480         | 7                     | 94.5                |
| 24         | 1.35% of the product of Example 7.<br>0.3% of the product of Example 32.                                                                                                                                                                                                      | 240         | 2                     | 98.5                |

Each of the above lubricants contained in addition to the specified dispersant additives 0.075% (as phosphorus) of a zinc dialkyl phosphorodithioate and 3 parts per million of a dimethyl silicone foam inhibitor. The lubricating oil was an SAE 30 mineral oil. The test results were evaluated according to two numerical standards:

(I) The piston cleanliness rating should be greater than 90.

(II) The number obtained by subtracting the top ring groove filling value from the piston cleanliness rating provides an overall indication of the efficacy of the test lubricant.

The piston cleanliness rating is based upon a scale of 1-100, 100 representing a perfectly clean piston.

Further illustration of the usefulness of the combination of additives of this invention was gained from a modified version<sup>1</sup> of the CRC-EX-3 Engine Test. This test is recognized in the field as an important test by which lubricants can be evaluated for use under light-duty service conditions. In this particular test the lubricant is used in the crankcase of a 1954 6-cylinder Chevrolet Powerglide engine for 144 hours under recurring cycling conditions, each cycle consisting of:

- 2 hours at an engine speed of  $500 \pm 25$  r.p.m. under zero load at an oil sump temperature of  $100^{\circ}$ - $125^{\circ}$  F.; air-fuel ratio of 10:1;
- 2 hours at an engine speed of  $2500 \pm 25$  r.p.m. under a load of 40 brake-horsepower at an oil sump temperature of  $240^{\circ}$ - $250^{\circ}$  F.; air-fuel ratio of 16:1.

After completion of the test, the engine is dismantled and various parts of the engine are examined for engine deposits. The lubricant dispersant addition agent is then rated according to (1) the extent of piston ring-filling, (2) the amount of sludge formed in the engine (on a scale of 80-0, 80 being indicative of no sludge and 0 being indicative of extremely heavy sludge), and (3) the total amount of engine deposits, i.e., sludge and varnish, formed

<sup>1</sup> Ordinarily this test lasts for 96 hours.

in the engine (on a scale of 100-0, 100 being indicative of no deposits and 0 being indicative of extremely heavy deposits). The results are summarized in Table III.

| Lubri-cant | Additives                                                                                                               | Percent Ring Filling | Sludge                                       | Total Engine Deposit |
|------------|-------------------------------------------------------------------------------------------------------------------------|----------------------|----------------------------------------------|----------------------|
| 25         | 0.9% of a product prepared as in Example 7 except that the polyisobutetyl radical contains an average of 61 carbons.    | 2                    | 77.9                                         | 97.0                 |
| 26         | 0.88% of the product of Example 20.<br>0.25% of the product of Example 21.                                              | 0                    | 76.5                                         | 94.9                 |
| 27         | 0.82% of the product prepared as in Example 7 except that the polyisobutetyl radical contains an average of 61 carbons. | 1                    | 77.3                                         | 95.7                 |
| 28         | 0.3% of the product of Example 19.                                                                                      | 1                    | 76.7                                         | 95.3                 |
| 29         | 0.68% of the product prepared as in Example 7 except that the polyisobutetyl radical contains an average of 61 carbons. | 6                    | 72.3                                         | 89.3                 |
| 30         | 0.82% of a product prepared as in Example 5.                                                                            | 1                    | 72.3                                         | 88.                  |
| 31         | 0.4% of a product of Example 25.                                                                                        | 2                    | 75.1                                         | 93.0                 |
| 32         | 1.34% of the product prepared as in Example 7 except that the polyisobutetyl radical contains an average of 61 carbons. | 5                    | 74.3                                         | 92.0                 |
| 33         | 0.44% of the product of Example 25.                                                                                     | 3                    | 74.2                                         | 92.5                 |
| 34         | 0.82% of the product of Example 5.                                                                                      | 7                    | 60.3                                         | 85.9                 |
| 35         | 0.2% of the product of Example 22.                                                                                      | 1                    | 75.4                                         | 92.                  |
| 36         | 0.82% of the product of Example 5.                                                                                      | 3                    | 73.0                                         | 88.0                 |
| 37         | 0.43% of the product of Example 29.                                                                                     | 55                   | 0.07% of normal calcium petroleum sulfonate. |                      |

What is claimed is:

1. A lubricating composition consisting essentially of a major proportion of a lubricating oil and
  - (a) from about 0.1 to about 10 percent by weight of an oil-soluble acylated amine prepared by the process which comprises mixing one equivalent of a substituted succinic compound selected from the class consisting of substituted succinic acids having the structural formula



and substituted succinic anhydrides having the structural formula



in which structural formulas R is a radical selected from the class consisting of large aliphatic hydrocarbon radicals having at least about 50 carbon atoms with at least about one-half an equivalent amount of an alkylene polyamine, and heating the resulting mixture, at a temperature above about 80° C. to effect acylation and remove the water formed thereby, and

(b) from about 0.05 to about 5.0 percent by weight as sulfate ash of an oil-soluble dispersant selected from the class consisting of alkaline earth metal petroleum sulfonates, alkaline earth metal alkyl-aromatic sulfonates, alkaline earth metal alkyl phenates and alkaline earth metal salts of phosphorus acids prepared from polymers of olefins having 2-30 carbon atoms said polymer having a molecular weight of at least about 750.

2. The lubricating composition of claim 1 characterized further in that the oil-soluble acylated amine of (a) is prepared by the process which comprises mixing one equivalent of a substituted succinic anhydride having the structural formula



in which structural formula R is a large aliphatic hydrocarbon radical having at least about 50 carbon atoms, with at least about one-half an equivalent amount of an ethylene polyamine having from 2 to about 6 amino groups, and heating the resulting mixture at a temperature above about 80° C. to effect acylation and remove the water formed thereby.

3. The lubricating composition of claim 1 characterized further in that the acylated amine of (a) is prepared by the process which comprises mixing one equivalent of a substituted succinic anhydride having the structural formula



in which structural formula R is a large aliphatic hydrocarbon radical having about 60 carbon atoms, with about one equivalent amount of an ethylene amine having from 2 to about 6 amino groups, and heating the resulting mixture at a temperature above about 80° C. to effect acylation and remove the water formed thereby.

4. The lubricating composition of claim 1 characterized further in that the oil-soluble dispersant of (b) is a carbonated basic barium sulfonate.

5. The lubricating composition of claim 1 characterized further in that the oil-soluble dispersant of (b) is a carbonated basic barium salt of a phosphorus acid prepared from a polymer of an olefin having 2-30 carbon atoms.

6. The lubricating composition of claim 1 characterized further in that the oil-soluble dispersant of (b) is a carbonated basic barium salt of a phosphorus acid prepared from a polymer of isobutylene.

7. The lubricating composition of claim 1 characterized further in that the oil-soluble dispersant of (b) is a carbonated basic barium salt of a phosphorus acid prepared by the steam-treatment of a chlorinated polyisobutylene-phosphorus trichloride reaction product.

8. The lubricating composition of claim 1 characterized further in that the oil-soluble dispersant of (b) is a carbonated basic barium salt of a phosphorus acid prepared by the steam-treatment of a polyisobutylene-phosphorus sulfide reaction product.

9. A lubricating composition consisting essentially of a major proportion of a mineral lubricating oil and (a) from about 0.1 to about 5.0 percent by weight of an oil-soluble acylated amine prepared by the process which comprises mixing one equivalent of a substituted succinic anhydride having the structural formula



in which structural formula R is a large aliphatic hydrocarbon radical having at least about 50 carbon atoms, with about one equivalent amount of an ethylene polyamine, and heating the resulting mixture at a temperature above about 80° C. to effect acylation and remove the water formed thereby, and

(b) from about 0.05 to about 10.0 percent by weight as sulfate ash of a barium salt of a phosphorus acid prepared from an isobutylene polymer having a molecular weight of about 1000.

10. The lubricating composition of claim 9 characterized further in that the oil-soluble dispersant of (b) is a carbonated basic barium salt of a phosphorus acid prepared by the steam-treatment of a polyisobutylene-phosphorus pentasulfide-sulfur reaction product.

11. A lubricating composition consisting essentially of a major proportion of a mineral lubricating oil and

(a) from about 0.1 to about 5 percent by weight of an oil-soluble acylated amine prepared by the process which comprises mixing one equivalent of a substituted succinic acid or anhydride in which the substituent is a large hydrocarbon radical having at least about 50 aliphatic carbon atoms with about one-half an equivalent amount of an ethylene polyamine having from about 2 to about 6 amino groups and heating the resulting mixture at a temperature above about 80° C. to effect acylation, and

(b) from about 0.5 to about 10 percent by weight of sulfate ash of a barium salt of a phosphorus acid prepared by the reaction of an olefin polymer having a molecular weight from about 750 to about 75,000 with phosphorus sulfide.

12. The lubricating composition of claim 11 characterized further in that the large hydrocarbon substituent of the substituted succinic acid or anhydride of (a) is a polyisobutene group having a molecular weight of from about 750 to about 11,000 and the oil soluble dispersant of (b) is a barium salt of a phosphorus acid prepared by the steam treatment of a polyisobutene-phosphorus pentasulfide reaction product.

#### References Cited by the Examiner

##### UNITED STATES PATENTS

|           |         |                 |       |            |
|-----------|---------|-----------------|-------|------------|
| 2,915,517 | 12/1959 | Le Suer         | ----- | 252-32.7 X |
| 3,001,981 | 9/1961  | Le Suer         | ----- | 252-32.7 X |
| 3,018,247 | 1/1962  | Anderson et al. | ----- | 252-51.5 X |
| 3,172,892 | 3/1965  | Le Suer et al.  | ----- | 252-51.5 X |
| 3,219,666 | 11/1965 | Norman et al.   | ----- | 252-51.5 X |
| 3,232,883 | 2/1966  | Le Suer         | ----- | 252-32.5   |

##### FOREIGN PATENTS

|    |         |        |         |
|----|---------|--------|---------|
| 65 | 541,926 | 6/1957 | Canada. |
|    | 570,814 | 2/1959 | Canada. |

DANIEL E. WYMAN, Primary Examiner.

70 P. P. GARVIN, Assistant Examiner.

UNITED STATES PATENT OFFICE  
CERTIFICATE OF CORRECTION

Patent No. 3,272,743

September 13, 1966

George R. Norman et al.

It is hereby certified that error appears in the above numbered patent requiring correction and that the said Letters Patent should read as corrected below.

Column 1, line 36, for "sludget" read -- sludge --; column 2, line 26, for "position" read -- positions --; line 47, for "substituent" read -- substituent --; line 67, for "component is" read -- component (a) is --; column 3, line 5, for "carboxylic" read -- carboxylate --; line 49, for "cases, it" read -- cases, however, it --; line 70, for "substituents" read -- substituent --; column 5, line 70, for "calcicm" read -- calcium --; column 6, line 60, for "phospohrus" read -- phosphorus --; column 9, line 37, for "squivalent" read -- equivalent --; line 41, for "azetropic" read -- azeotropic --; line 48, for "parts of" read -- parts by weight of --; column 10, line 20, for "dis-(1,2-propylene)" read -- di-(1,2-propylene --; line 34, for "2.5" read -- 2.55 --; line 47, for "12-174° C." read -- 112-174° C. --; line 62, for "temperautre" read -- temperature --; lines 63 and 64, for "temperature and the" read -- temperature the --; column 14, line 49, for "excect" read -- except --; line 67, for "0.56%" read -- 0.57% --; column 15, line 16, for "0.27%" read -- 0.25% --; column 16, line 28, for "as Example" read -- as in Example --; line 30, for "88." read -- 88.5 --; line 49, for "92." read -- 92.6 --.

Signed and sealed this 8th day of October 1968.

(SEAL)

Attest:

EDWARD M.FLETCHER,JR.  
Attesting Officer

EDWARD J. BRENNER  
Commissioner of Patents